

-M

UNITED STATES PATENT OFFICE

CHARLES C. NEIGHBORS, OF CHICAGO, ILLINOIS, ASSIGNOR TO WESTERN ELECTRIC COMPANY, INCORPORATED, OF NEW YORK, N. Y., A CORPORATION OF NEW YORK  
MAGNETIC MATERIAL, METHOD OF MAKING THE SAME, AND ARTICLES MADE THEREFROM

No Drawing.

Application filed December 31, 1930. Serial No. 505,956.

This invention relates to a magnetic material, a method of making the same, and articles made therefrom, and more particularly to a material for making magnetic core parts of the compressed dust type for use in telephonic communicating systems, to a method of making such material, and to magnetic core parts made from such material.

10 An object of the invention is to produce a magnetic material which will withstand high forming pressures and high treating temperatures, is non-corrosive, non-oxidizing, has a low affinity for water, and from which 15 magnetic cores may be produced of satisfactory mechanical and electrical properties and having very low water absorbing characteristics.

In one embodiment of the invention, the 20 magnetic material consists of a magnetic alloy in finely divided form, the particles of which are insulated from each other by an insulating composition which includes a water-soluble organic acid, such as tartaric acid, together with additional ingredients such as sodium silicate, talc, and kaolin. The insulating composition is intimately mixed with the particles of the alloy, and the resulting material is heated to dryness and 30 sifted, after which the material is pressed into cores suitable for use in telephonic communicating systems.

Other objects and advantages of the invention will become apparent from the following description.

In practicing the present invention, the magnetic material is preferably prepared from a brittle alloy containing nickel and iron, with or without the addition of other 40 constituents, and commonly known as "perm-alloy". The alloy may be prepared in the manner described in Patent No. 1,669,649 issued May 15, 1928 to C. P. Beath and H. M. E. Heinicke, wherein approximately 45 81 parts of nickel and 19 parts of iron are melted together in an oxidizing atmosphere, the resulting alloy being poured into a mold. The alloy thus prepared is rolled while hot into relatively thin slabs which are quenched 50 rapidly to produce a fine crystalline struc-

ture which is desirable since the disintegration of the material takes place at the crystal boundaries, and consequently the smaller the size of the crystals the finer the dust which can be produced therefrom. The slabs are then reduced to a finely divided form in any suitable manner and the finely divided alloy is subsequently reduced to a dust by pulverizing it in an attrition or ball mill.

The dust from the attrition or ball mill 55 is then sifted and the portion passing through a 120-mesh screen is placed in a closed container and annealed at a temperature of approximately 885° C. The annealed dust is removed from the container in the form of a cake, which is again reduced to a powder by crushing it in a rotary crusher and subsequently grinding it in an attrition mill, the ground dust is again sifted through a 120-mesh screen and the dust passing the screen 60 is then mixed with the insulating composition described below. It should be understood, however, that the present invention is independent of the particular magnetic metal or alloy employed, and of the manner of preparing the metal or alloy. The term "magnetic metal", as used herein, is therefore intended to include any magnetic metal or alloy of metals suitable for use in connection with the present invention, regardless of its composition or method of preparation.

As an example of an insulating composition suitable for the purposes of the present invention, the following formula is given:

|                 | Pounds              |
|-----------------|---------------------|
| Tartaric acid   | .30                 |
| Sodium silicate | 1.05                |
| Powdered talc   | .75                 |
| Kaolin          | .75                 |
| Water           | 12.00 <sup>90</sup> |

The ratio of acid to sodium silicate as given in the above formula is 1:3½, but may range from 1:3 to 1:8 or upwards, the effectiveness of the insulation decreasing 65 somewhat as the ratio of acid to sodium silicate decreases from that given in the above formula. The ratio of the solid materials (talc and kaolin) to the water-soluble materials (acid and sodium silicate) may be va- 70

ried widely, as may also the ratio of water to the other ingredients, the water being used merely to dissolve the water-soluble materials and to give the desired consistency to the mixture of insulating composition and dust.

The kaolin specified in the above formula is a binder and has the function of preventing cracks in the finished core parts, in addition to being a rather effective insulating material. In certain cases it may be omitted, depending upon the characteristics desired in the finished core parts.

The permalloy dust is thoroughly mixed with the insulating composition, the ratio between the dust and the insulating composition being determined by the permeability desired, which varies with the particular use to which the finished cores are to be put. For most purposes, the amounts specified in the above formula would be mixed with about 100 pounds of dust. The entire mass is then evaporated to a condition of complete dryness in order to obtain the maximum insulation resistance, and is stirred constantly to prevent caking and to insure a thorough coating of the individual dust particles. To obtain a complete drying of the magnetic material its temperature may be raised to 120° C., and even much higher temperatures may be used without injury to the material. The material after being thoroughly dried has a very low affinity for water, so that no special protection need be provided against the absorption of water by the material.

The insulated dust is then sifted through a 16-mesh screen, placed in a mold and compressed into core parts under a pressure of approximately 200,000 pounds per square inch. The core parts are then transferred to an annealing furnace where they are annealed to relieve the internal stresses set up by the pressing operation and thereby to produce a core having low hysteresis loss. The annealing temperature used is preferably about 565° C., but a temperature as high as 620° C. may be used without destroying the effectiveness of the insulation. Where a temperature of 565° is used, the core parts are preferably raised to that temperature in about eleven minutes and maintained at such temperature for about three minutes. If higher annealing temperatures are used the time should of course be proportionately shortened, and vice versa.

The drying and annealing temperatures apparently drive off substantially all of the volatile constituents of the material, including the organic acid, in the form of gases, with the result that the annealed core parts contain only the end-products of the heating process, and contain no water-absorbent substances. This makes it unnecessary to wash and dry the core parts after anneal-

ing to remove such water-absorbent substances. The tartaric acid used is a very weak oxidizing agent, and since it volatilizes at a relatively low temperature very little oxidation of the metal takes place during the annealing operation. Such oxidation may be objectionable in some cases since it appears to affect unfavorably the magnetic qualities of the finished cores.

One or more core parts thus formed are then used to constitute a core to which the usual toroidal winding is applied to form a loading coil, the number of core parts used depending upon the electrical characteristics of the circuit with which the loading coil is to be associated.

In place of the tartaric acid specified in the above formula, any other suitable water-soluble organic acid may be used, although it is preferred to use a non-corrosive, non-irritating, non-oxidizing organic acid and one which leaves a non-hygroscopic residue, such as tartaric, lactic and citric acids. Other suitable acids which may be used are succinic, oxalic, and malonic acids.

The invention is not limited to the embodiments above described, but may be varied widely within the scope of the following claims:

What is claimed is:

1. A magnetic material suitable for producing magnetic cores, comprising a finely divided magnetic metal, and an insulating composition mixed therewith and including a water-soluble organic acid.

2. A magnetic material suitable for producing magnetic cores, comprising finely divided particles of a magnetic metal, and an insulating composition intimately associated with said particles and including tartaric acid.

3. A magnetic material suitable for producing magnetic cores, comprising finely divided particles of a magnetic metal, and an insulating composition intimately associated with said particles and including lactic acid.

4. A magnetic material suitable for producing magnetic cores, comprising finely divided particles of a magnetic metal, and an insulating composition intimately associated with said particles and including citric acid.

5. A composition of matter comprising finely divided magnetic metal, a water-soluble organic acid, sodium silicate, and a ceramic binding material.

6. A composition of matter comprising the following ingredients in about the following proportions: finely divided magnetic metal, 100 parts; tartaric acid, 0.30 parts; sodium silicate, 1.05 parts; powdered talc, 0.75 parts; and kaolin, 0.75 parts.

7. A magnetic material comprising finely divided magnetic metal, and an insulating composition forming a coating on the par-

- 5 ticles of metal and including the end-products obtained by heating a mixture of a water-soluble organic acid, sodium silicate, and talc, to a temperature above 400° C.
- 5 8. A method of producing a magnetic material which comprises mixing together a finely divided magnetic metal, a water-soluble organic acid, sodium silicate, a ceramic binding material, and water, and evaporating the resulting mixture to complete dryness.
- 15 9. A method of producing a magnetic material which comprises mixing a finely divided magnetic metal with an insulating composition including a water-soluble organic acid, sodium silicate, a ceramic material and water, and heating the resulting mixture to drive off substantially all of the volatile constituents thereof.
- 20 10. A method of making a magnetic material which comprises mixing a finely divided magnetic metal with an insulating composition made up of a water-soluble organic acid, sodium silicate, a ceramic material, and water, heating the resulting mixture to dry it completely, and simultaneously stirring the mixture to prevent it caking and to cause the insulating composition to coat the particles of magnetic metal.
- 30 11. A method of making a magnetic material which comprises mixing a finely divided magnetic metal with an insulating composition made up of tartaric acid, sodium silicate, a ceramic material, and water, heating the resulting mixture to dry it completely, and simultaneously stirring the mixture to prevent it caking and to cause the insulating composition to coat the particles of magnetic metal.
- 40 12. A method of making a magnetic material which comprises mixing a finely divided magnetic metal with an insulating composition made up of lactic acid, sodium silicate, a ceramic material, and water, heating the resulting mixture to dry it completely, and simultaneously stirring the mixture to prevent it caking and to cause the insulating composition to coat the particles of magnetic metal.
- 50 13. A method of making a magnetic material which comprises mixing a finely divided magnetic metal with an insulating composition made up of citric acid, sodium silicate, a ceramic material, and water, heating the resulting mixture to dry it completely, and simultaneously stirring the mixture to prevent it caking and to cause the insulating composition to coat the particles of magnetic metal.
- 60 14. A method of making a magnetic material which comprises mixing a finely divided magnetic metal with an insulating composition comprising a water-soluble organic acid and a binder, heating and agitating the resulting mixture to dry it completely in the form of a dust, compressing the dust to cause the particles thereof to cohere and form a solid mass, and annealing the mass to relieve internal stresses and to drive off the volatile constituents of the mass.
- 70 15. A magnetic core part formed of finely divided magnetic metal and an insulating composition forming a coating on the particles of magnetic metal and including the end-products obtained by heating a mixture of a water-soluble organic acid, sodium silicate, and talc, to a temperature above 400° C.
- 75 16. A magnetic core part formed of finely divided magnetic metal and an insulating composition forming a coating on the particles of magnetic metal and including the end-products obtained by heating a mixture of tartaric acid, sodium silicate, and talc, to a temperature above 400° C.
- 80 17. A magnetic core part formed of finely divided magnetic metal and an insulating composition forming a coating on the particles of magnetic metal and including the end-products obtained by heating a mixture of lactic acid, sodium silicate, and talc, to a temperature above 400° C.
- 85 18. A magnetic core part formed of finely divided magnetic metal and an insulating composition forming a coating on the particles of magnetic metal and including the end-products obtained by heating a mixture of citric acid, sodium silicate, and talc, to a temperature above 400° C.
- 90 19. A magnetic core part formed of finely divided magnetic metal and an insulating composition coating the particles of magnetic metal and comprising the products obtained by heating a mixture of a water-soluble organic acid, sodium silicate, and a ceramic binder, to a temperature of about 565° C.
- 100 20. A magnetic core part formed of finely divided particles of magnetic metal coated with an insulating composition comprising the products obtained by heating a mixture of a water-soluble organic acid, sodium silicate, and a ceramic binder, to an annealing temperature, said particles being held together in fixed relation by an autogenous bond created by compression.
- 110 21. A magnetic core part formed of finely divided particles of magnetic metal coated with an insulating composition comprising the products obtained by heating a mixture of a water-soluble organic acid, sodium silicate, talc, kaolin, and water, to a temperature sufficiently high to dry the mixture completely, said particles being held together in fixed relation by an autogenous bond created by compression.
- 120 22. A magnetic core part comprising finely divided particles of magnetic metal and an insulating composition comprising the products obtained by heating a mixture of .30 parts of tartaric acid, 1.05 parts of sodium
- 125
- 130

silicate, .75 parts of powdered talc, .75 parts of kaolin, and 12 parts of water to each 100 parts of metal, to a temperature substantially above 100° C.

5 23. A magnetic core part formed of finely divided magnetic metal and an insulating composition forming a coating on the particles of magnetic metal and consisting of a non-hygroscopic residue of an evaporated 10 mixture of insulating material and a water-soluble organic acid.

24. A magnetic core part formed of finely divided magnetic metal and an insulating composition forming a coating on the particles of magnetic metal and consisting of a non-hygroscopic residue of an evaporated 15 mixture of a water-soluble organic acid, sodium silicate, and a ceramic binding material.

20 In witness whereof, I hereunto subscribe my name this 20th day of December, A. D. 1930.

CHARLES C. NEIGHBORS.

25

30

35

40

45

50

55

60

65